

Jan. 12, 1960

G. C. JOHNSON ET AL

2,921,017

PROCESS OF PRODUCING DESULFURIZED COKE FROM PETROLEUM

Filed Feb. 13, 1957



*Fig. 2*

EFFECT OF COKING TEMPERATURE  
ON SULFUR CONTENT OF COKE.



*Fig. 3*

EFFECT OF TEMPERATURE ON  
DEGREE OF DESULFURIZATION



INVENTORS

George C. Johnson  
Sigmund J. Lukasiewicz  
Charles A. Higgett

ATTORNEY

1

2,921,017

## PROCESS OF PRODUCING DESULFURIZED COKE FROM PETROLEUM

George C. Johnson and Sigmund J. Lukasiewicz, Woodbury, N.J., assignors to Socony Mobil Oil Company, Inc., a corporation of New York

Application February 13, 1957, Serial No. 639,945

10 Claims. (Cl. 208—106)

This invention relates to the production of petroleum coke of low sulfur content from petroleum residua of high sulfur content.

In the manufacture of petroleum products the customary practice involves the separation of the crude petroleum oil into various fractions or cuts having limited boiling range, thereby providing products suitable for specific purposes. The prime products are naphtha and the distillate fuel oils useful as heating oil and diesel fuels. However, many other useful products are obtained from petroleum, including a hard brittle coke having a low ash content.

After the light products have been removed from the crude oil, there remains a heavy viscous liquid which is characterized as residuum. In one form of the conventional coking process the residuum is charged to a distillation tower with the overhead from a coker and the mixture separated into gas, gasoline, gas oil and residuum. The residuum is removed from the bottom of the distillation tower, pumped through a furnace and charged to the coker. A typical coking temperature is about 900° F. and a typical pressure is 60 p.s.i.g. The finished coke is very much in demand and the market is continually increasing. Petroleum coke is a major raw material for making anodes for the aluminum industry. Anodes for use in this industry should be low in ash and sulfur.

As crude sources are being continually exhausted, more and more crudes having a high sulfur content are being charged to processing equipment throughout the world to provide desired products. Among these are such crudes as Santa Maria Valley, West Cat Canyon, Kuwait and Slaughter. These crudes yield coke containing more than 2 percent sulfur and this amount is excessive for many uses, such as, for example, the electrodes in the aluminum industry.

We have found that the sulfur content of petroleum coke can be suitably reduced by grinding the coke and mixing it with powdered sodium carbonate, heating the mixture to a temperature of about 1400° F. for a short period of time and then water washing the product to provide a desulfurized coke. The product coke is a commercially acceptable coke.

This invention involves an improved process in which the powdered sodium carbonate is mixed with the residuum before the coking operation and the coking conditions are changed sufficiently to effect the coking and desulfurization in a single operation. The coke produced is provided in commercially acceptable form.

The object of this invention is to provide a process for producing a low sulfur content coke product from a high sulfur content crude.

A further object of this invention is to provide a simplified process for directly producing a low sulfur content coke from a petroleum which is high in sulfur.

These and other objects will become clear from a review of the following detailed description of the invention.

Figure 1 is a block diagram of the improved process which is used in the following detailed description.

2

Figure 2 is a plot of weight percent sulfur in the coke produced versus coking temperature for a given high sulfur residuum.

Figure 3 shows the effect of temperature on the desulfurization of coke.

Referring to Figure 1, petroleum residuum obtained from atmospheric or vacuum topping of the crude is charged to the distillation tower 10 through the path 11. Hot vapors from the coker 18 are introduced into the tower 10 through the path 9 to heat exchange with the residuum and raise the temperature of the residuum. The gas and gasoline vis., the lightest products, are removed overhead through the path 12. A somewhat heavier cut, such as a gas oil, is removed from the distillation tower 10 through the path 13. The remaining heavy product or residuum is removed from the bottom of the distillation tower 10 through the path 14 and introduced into a mixer 15. The sodium carbonate is preferably crushed or powdered first and then introduced into the mixer 15 through the path 16. The mixture of residuum and sodium carbonate is then transferred through the path 17 to the calciner coker 18.

Although coking will generally take place at a satisfactory rate at about 900° F. and 60 p.s.i., the temperature in the calciner coker is maintained substantially above 900° F. in this process, for example, 1400° F. being most suitable. Hot gases can be used to heat the calciner coker to this temperature. After a suitable period of time, the coke is removed from the calciner coker and transferred through the path 19 to the washer 20. Water is introduced into the washer 20 through the path 21. The water solution is removed through the path 22 and finally the desulfurized product coke is removed through the path 23.

The effect of coking temperature upon the sulfur content of the coke is shown on Figure 2. It is seen that correct temperature is important and that lowest sulfur content occurs at or about 1400° F. At lower temperatures or higher temperatures the product coke contains more sulfur. The graph shown on Figure 2 was prepared from data obtained by coking a residuum containing about 6.41% sulfur. The 1400° F. temperature is also the optimum in the desulfurization of coke, as shown in Figure 3.

The amount of sodium carbonate to be used depends upon the amount of sulfur present in the residuum. The usual operating range is about 0.7 to 7.2 lb. sodium carbonate for each pound of sulfur which would be present in the coke produced from the residuum if no sodium carbonate were present. For example, if the residuum yields 14% of coke containing 5.16% sulfur, the usual amount of sodium carbonate used would be 0.51 to 5.2 lb. per 100 lb. of residuum.

The optimum operating conditions are tabulated as follows:

|                                  | Preferred Range                                                                              | Broad Range                                                                                          |
|----------------------------------|----------------------------------------------------------------------------------------------|------------------------------------------------------------------------------------------------------|
| Temperature, ° F. ....           | 1,300-1,500.....                                                                             | 1,100-1,800.....                                                                                     |
| Pressure ..... Atm. ....         | 0.1 atm.-50 atm. ....                                                                        | 1 min.-4 hrs. ....                                                                                   |
| Time at Reaction Temp. ....      | 15-60 min. ....                                                                              | 0.7 or greater lbs./lb. of sulfur in coke made without Na <sub>2</sub> CO <sub>3</sub> present. .... |
| Amount of Sodium Carbonate. .... | 0.7-7.2 lb./lb. of sulfur in coke made without Na <sub>2</sub> CO <sub>3</sub> present. .... | 1 lb. of sulfur in coke made without Na <sub>2</sub> CO <sub>3</sub> present. ....                   |

While the process is primarily adapted for use in preparing low sulfur content coke from liquid petroleum residuum, it can also be used on residuum obtained from shale or from tar sands. The invention is particularly useful when the residuum without carbonate would yield a coke containing at least 2% sulfur.

The invention was tested using 72% Santa Maria residuum with sodium carbonate. Table I below shows the results:

As an alternative process the coking and desulfurization of the residuum may be carried out in two steps. For example, the residuum may be mixed with the sodium

Table I

| Run No. | Charge                          | Material Added                  | Amount of Material Added, Wt. Percent | Coking Temp., °F. | Time, Hr. | Sulfur in Charge, Wt. Percent | Sulfur in Product Coke, Wt. Percent | Coke Yield, Wt. Percent |
|---------|---------------------------------|---------------------------------|---------------------------------------|-------------------|-----------|-------------------------------|-------------------------------------|-------------------------|
| 38      | 72% Santa Maria Valley Residuum | Na <sub>2</sub> CO <sub>3</sub> | 20                                    | 916               | 1         | 6.41                          | 5.16                                | 22                      |
| 43      | do                              | Na <sub>2</sub> CO <sub>3</sub> | 20                                    | 1,200             | 1         | 6.41                          | 8.27                                | 17                      |
| 44      | do                              | Na <sub>2</sub> CO <sub>3</sub> | 20                                    | 1,409             | 1         | 6.41                          | 2.67                                | 14                      |
| 48      | do                              | Na <sub>2</sub> CO <sub>3</sub> | 20                                    | 1,404             | 1         | 6.41                          | 2.63                                | 14                      |
| 49      | do                              | Na <sub>2</sub> CO <sub>3</sub> | 20                                    | 1,488             | 1         | 6.41                          | 2.96                                | 12                      |
| 62      | do                              | Na <sub>2</sub> CO <sub>3</sub> | 5                                     | 1,401             | 1         | 6.41                          | 3.15                                | 12                      |

While sodium carbonate is a suitable material useful for desulfurization in the process as described above, other alternative materials are available. These include sodium bicarbonate, sodium sesquicarbonate, sodium carbonate monohydrate, sodium carbonate heptahydrate, sodium carbonate decahydrate and sodium hydroxide. These materials have been tested with coke obtained from different crude sources and at different operating conditions, with the result that desulfurization to varying degrees has been obtained.

Table II, which follows hereinafter, shows the results of these tests.

25 carbonate and coked at a temperature of 900° F. or thereabouts. This provides a good mixture of the sodium carbonate and coke. Then the mixture is transferred to a separate vessel where the temperature may be raised to 1400° F. to complete the coking and desulfurization. The two steps may be carried out in separate vessels or alternatively, the two stages may be carried out successively in a single vessel by raising the temperature from 900° F. to 1400° F. Afterwards, the desulfurized coke product is washed with water to remove salts, providing a finished commercially marketable coke. Suitable con-

Table II

| Run | Charge                  | Original Coking Temp., °F. | Mesh Size of Coke | Material Added                                      | Amt. of Material Added, Wt. Percent | Method of Mixing | Re-coking Temp., °F. | Time, Hours | Sulfur in Charge, Wt. Percent | Sulfur in Product, Wt. Percent | Sulfur Removal, Wt. Percent | Coke Yield, Wt. Percent |
|-----|-------------------------|----------------------------|-------------------|-----------------------------------------------------|-------------------------------------|------------------|----------------------|-------------|-------------------------------|--------------------------------|-----------------------------|-------------------------|
| 8   | Houk Coke <sup>1</sup>  | 900                        | 60-100            | None                                                | 0                                   | Impreg.          | 1,390                | 1.0         | 7.01                          | 6.37                           | 9                           | 88                      |
| 33  | do                      | 900                        | 60-100            | Na <sub>2</sub> CO <sub>3</sub>                     | 5                                   | Impreg.          | 1,405                | 1.0         | 7.01                          | 5.57                           | 21                          | 86                      |
| 30  | do                      | 900                        | 60-100            | Na <sub>2</sub> CO <sub>3</sub>                     | 10                                  | Impreg.          | 1,405                | 1.0         | 7.01                          | 3.23                           | 54                          | 85                      |
| 31  | do                      | 900                        | 60-100            | Na <sub>2</sub> CO <sub>3</sub>                     | 20                                  | Impreg.          | 1,417                | 1.0         | 7.01                          | 3.15                           | 55                          | 85                      |
| 32  | do                      | 900                        | 60-100            | Na <sub>2</sub> CO <sub>3</sub>                     | 20                                  | Impreg.          | 925                  | 1.0         | 7.01                          | 6.97                           | 1                           | 96                      |
| 34  | do                      | 900                        | 60-100            | Na <sub>2</sub> CO <sub>3</sub>                     | 20                                  | Impreg.          | 1,204                | 1.0         | 7.01                          | 4.45                           | 37                          | 88                      |
| 75  | Santa Maria Valley Coke | 916                        | 60-100            | None                                                | 0                                   | Impreg.          | 1,404                | 1.0         | 5.57                          | 4.83                           | 13                          | 92                      |
| 51  | do                      | 1,000                      | 60-100            | Na <sub>2</sub> CO <sub>3</sub>                     | 20                                  | Mixing           | 1,215                | 1.0         | 5.64                          | 4.03                           | 29                          | 94                      |
| 63  | do                      | 1,000                      | 60-100            | Na <sub>2</sub> CO <sub>3</sub>                     | 20                                  | do               | 1,227                | 4.0         | 5.64                          | 2.77                           | 51                          | 92                      |
| 45  | do                      | 1,000                      | 60-100            | Na <sub>2</sub> CO <sub>3</sub>                     | 20                                  | do               | 1,402                | 0.5         | 5.64                          | 3.09                           | 45                          | 91                      |
| 36  | do                      | 1,000                      | 60-100            | Na <sub>2</sub> CO <sub>3</sub>                     | 20                                  | do               | 1,405                | 1.0         | 5.64                          | 2.88                           | 49                          | 91                      |
| 37  | do                      | 1,000                      | 60-100            | Na <sub>2</sub> CO <sub>3</sub>                     | 20                                  | Impreg.          | 1,410                | 1.0         | 5.64                          | 2.85                           | 50                          | 90                      |
| 47  | do                      | 1,000                      | 60-100            | Na <sub>2</sub> CO <sub>3</sub>                     | 20                                  | Mixing           | 1,418                | 4.0         | 5.64                          | 2.88                           | 49                          | 95                      |
| 69  | do                      | 916                        | 60-100            | Na <sub>2</sub> CO <sub>3</sub>                     | 10                                  | do               | 1,400                | 1.0         | 5.57                          | 2.92                           | 48                          | 89                      |
| 46  | do                      | 1,000                      | 60-100            | Na <sub>2</sub> CO <sub>3</sub>                     | 20                                  | do               | 1,527                | 1.0         | 5.64                          | 3.54                           | 37                          | 95                      |
| 40  | do                      | 1,000                      | 60-100            | Na <sub>2</sub> CO <sub>3</sub>                     | 20                                  | do               | 1,600                | 1.0         | 5.64                          | 3.45                           | 39                          | 96                      |
| 41  | do                      | 1,000                      | 60-100            | Na <sub>2</sub> CO <sub>3</sub>                     | 20                                  | do               | 1,763                | 1.0         | 5.64                          | 3.88                           | 31                          | 98                      |
| 52  | do                      | 1,000                      | 20-60             | Na <sub>2</sub> CO <sub>3</sub>                     | 20                                  | do               | 1,408                | 1.0         | 5.64                          | 3.32                           | 41                          | 95                      |
| 54  | do                      | 1,000                      | 100-200           | Na <sub>2</sub> CO <sub>3</sub>                     | 20                                  | do               | 1,408                | 1.0         | 5.64                          | 2.70                           | 52                          | 90                      |
| 50  | do                      | 1,000                      | <100              | Na <sub>2</sub> CO <sub>3</sub>                     | 20                                  | do               | 1,407                | 1.0         | 5.64                          | 2.32                           | 59                          | 89                      |
| 53  | Product of Runs, 45, 47 | 2,140                      | 60-100            | Na <sub>2</sub> CO <sub>3</sub>                     | 20                                  | do               | 1,407                | 1.0         | 2.98                          | 1.83                           | 39                          | 97                      |
| 60  | Santa Maria Valley Coke | 1,000                      | 60-100            | Trona <sup>2</sup>                                  | 28.4                                | do               | 1,410                | 1.0         | 5.64                          | 1.85                           | 67                          | 91                      |
| 65  | do                      | 1,000                      | 60-100            | NaHCO <sub>3</sub>                                  | 20                                  | do               | 1,408                | 1.0         | 5.64                          | 3.51                           | 38                          | 92                      |
| 68  | do                      | 1,000                      | 60-100            | Na <sub>2</sub> CO <sub>3</sub> .H <sub>2</sub> O   | 23.4                                | do               | 1,400                | 1.0         | 5.64                          | 2.79                           | 51                          | 89                      |
| 57  | Kuwait Coke             | 1,036                      | 60-100            | Na <sub>2</sub> CO <sub>3</sub>                     | 23.4                                | do               | 1,410                | 1.0         | 7.29                          | 2.63                           | 64                          | 91                      |
| 71  | Santa Maria Valley Coke | 916                        | 60-100            | NaHCO <sub>3</sub>                                  | 31.7                                | do               | 1,400                | 1.0         | 5.57                          | 2.75                           | 51                          | 91                      |
| 70  | do                      | 916                        | 60-100            | Trona <sup>4</sup>                                  | 28.4                                | do               | 1,403                | 1.0         | 5.57                          | 2.56                           | 54                          | 92                      |
| 74  | do                      | 916                        | 60-100            | Trona <sup>3</sup>                                  | 28.4                                | do               | 1,405                | 1.0         | 5.57                          | 1.99                           | 64                          | 90                      |
| 70  | do                      | 916                        | 60-100            | Trona <sup>5</sup>                                  | 28.4                                | do               | 1,404                | 1.0         | 5.57                          | 2.59                           | 54                          | 91                      |
| 77  | do                      | 916                        | 60-100            | Trona <sup>6</sup>                                  | 28.4                                | do               | 1,406                | 1.0         | 5.57                          | 2.80                           | 59                          | 89                      |
| 78  | do                      | 916                        | 60-100            | Na <sub>2</sub> CO <sub>3</sub> .10H <sub>2</sub> O | 54.0                                | do               | 1,402                | 1.0         | 5.57                          | 2.35                           | 58                          | 90                      |
| 55  | do                      | 1,000                      | 60-100            | NaCl                                                | 20                                  | do               | 1,411                | 1.0         | 5.64                          | 5.06                           | 10                          | 92                      |
| 56  | do                      | 1,000                      | 60-100            | CaO                                                 | 20                                  | do               | 1,413                | 1.0         | 5.64                          | 4.67                           | 17                          | 95                      |
| 66  | do                      | 1,000                      | 60-100            | NaOH                                                | 20                                  | Impreg.          | 1,413                | 1.0         | 5.64                          | 1.17                           | 79                          | 90                      |

<sup>1</sup> This is a West Cat Canyon, California crude.

<sup>2</sup> Average of 1402 and 1418° F.

<sup>3</sup> Sodium sesquicarbonate—lab. preparation.

<sup>4</sup> Sodium sesquicarbonate—commercial purified needles.

<sup>5</sup> Sodium sesquicarbonate—60-100 mesh (commercial).

<sup>6</sup> Sodium sesquicarbonate—commercial below 200 mesh.

ditions for conducting the process in two stages are as follows:

|                        | Preferred                                                 | Broad                 |
|------------------------|-----------------------------------------------------------|-----------------------|
| Temp., ° F., 1st stage | 830-930                                                   | 800-1,000.            |
| Pressure, 1st stage    | 60 lbs./sq. in.                                           | 1/10th atm.-50 atm.   |
| Sodium Carbonate       | 0.7-7.2 lb./lb. of sulfur in coke made without carbonate. | More than 0.7 lb./lb. |
| Temp., ° F., 2nd stage | 1,300-1,500                                               | 1,100-1,800.          |
| Time, 2nd stage        | 15-60 min.                                                | 1 min.-4 hrs.         |

The sodium carbonate is preferably used in the form of a fine powder although small lumps can be used successfully. The coke from the low temperature stage should not be water-washed nor removed from the coker by hydraulic means, otherwise, sodium carbonate will be lost. The pressure is usually about atmospheric pressure in the high temperature step. The coke from the high temperature stage is preferably crushed before washing but may be used as lumps with consequent added difficulty in removing the salts by washing with water.

Table III illustrates the invention as a two-stage process.

Table III

| Run No. | Charge                          | Sulfur in Charge, Wt. Percent | Material Added                  | Amt. of Material Added, Wt. Percent | Temperature 1st Stage        | Sulfur in Product Coke, Wt. Percent | Coke Yield, Wt. Percent |
|---------|---------------------------------|-------------------------------|---------------------------------|-------------------------------------|------------------------------|-------------------------------------|-------------------------|
| 67      | Santa Maria Valley Crude        | 4.65                          | None                            |                                     | 916                          | 5.57                                | 12.6                    |
| 35      | do                              | 4.65                          | None                            |                                     | 930                          | 5.64                                | 10                      |
| 64A     | 72% Santa Maria Valley Residuum | 6.41                          | Na <sub>2</sub> CO <sub>3</sub> | 6                                   | 880                          |                                     |                         |
| Run No. | Charge                          | Sulfur in Charge, Wt. Percent | Material Added                  | Amt. of Material Added, Wt. Percent | Coking Temp., ° F. 2nd Stage | Sulfur in Product Coke, Wt. Percent | Coke Yield, Wt. Percent |
| 75      | Coke From Run 67                | 5.57                          | None                            | 0                                   | 1,404                        | 4.83                                | 92                      |
| 36      | Coke From Run 35                | 5.64                          | Na <sub>2</sub> CO <sub>3</sub> | 20                                  | 1,405                        | 2.88                                | 91                      |
| 64B     | Coke From Run 64A               |                               | None                            |                                     | 1,405                        | 3.43                                | 27                      |

\* Reflux liquid returned to coking operation.  
† Step #1 plus Step #2.

We claim:

1. The method of producing a low sulfur petroleum coke from a high sulfur petroleum residuum which comprises the steps of mixing with the residuum a material selected from the group consisting of sodium carbonate, sodium bicarbonate, sodium sesquicarbonate, sodium carbonate monohydrate, sodium carbonate heptahydrate, sodium carbonate decahydrate and sodium hydroxide and subjecting the mixture to high temperature coking conditions to produce a petroleum coke, washing the coke formed to effect removal of sulfur salts, whereby a petroleum coke is produced having a substantially reduced sulfur content from that of the residuum from which it is formed.

2. Claim 1 further characterized in that the coking temperature is about 1100-1800° F.

3. Claim 1 further characterized in that the coking temperature is about 1300-1500° F.

4. The method of producing a low sulfur petroleum coke from a high sulfur petroleum residuum which comprises the steps of mixing with the residuum at least a sufficient amount of sodium carbonate in particle form, subjecting the mixture to an advanced temperature for a sufficient period of time to produce a petroleum coke having a substantially lower sulfur content by weight than would be provided if the sodium carbonate were not present, and washing the coke formed to effect removal of sulfur-containing salts from the coke.

5. Claim 4 further characterized in that the coking

temperature is about 1100-1800° F. and the reaction time is about 1 minute-4 hours and the amount of sodium carbonate is 0.7 or greater lbs./lb. of sulfur in the coke made without sodium carbonate present and the pressure during reaction is about 0.1 atmosphere-50 atmospheres.

6. Claim 4 further characterized in that the coking temperature is about 1300-1500° F. and the reaction time is about 15-60 minutes and the amount of sodium carbonate is about 0.7-7.2 lb./lb. of sulfur in coke made without sodium carbonate present and the pressure is about atmospheric.

7. The method of producing a low sulfur petroleum coke from a high sulfur petroleum residuum which comprises the steps of mixing with the residuum a material selected from the group consisting of sodium carbonate, sodium bicarbonate, sodium sesquicarbonate, sodium carbonate monohydrate, sodium carbonate heptahydrate and sodium carbonate decahydrate, subjecting the mixture to low temperature coking conditions and then subjecting the mixture to a substantially higher temperature, sufficient to effectively reduce the sulfur content of the finished coke below the amount which would be present in the coke if the carbonate were not used, and washing

the product to effect removal of salts from the coke product.

8. Claim 7 further characterized in that the mixture is first heated to a temperature of about 800-1000° F., the pressure being maintained at about  $\frac{1}{10}$  atmosphere-50 atmospheres, the amount of carbonate being at least 0.7 lb./lb. of sulfur in coke made without carbonate, and the material is then heated to about 1100-1800° F. for a period about 1 minute-4 hours, whereby a coke is produced of substantially reduced sulfur content.

9. Claim 7 further characterized in that the mixture is first heated to a temperature of about 800-930° F., the pressure is maintained at about 60 p.s.i., the amount of carbonate is about 0.7-7.2 lb./lb. of sulfur in coke made without carbonate, and the material is then heated to about 1300-1500° F. for about 15-60 minutes, whereby a coke is produced of substantially reduced sulfur content.

10. Claim 9 further characterized in that the carbonate material is sodium carbonate.

#### References Cited in the file of this patent

#### UNITED STATES PATENTS

70 2,768,939 Mason et al. Oct. 30, 1956  
2,814,588 Hutchings Nov. 26, 1957

#### OTHER REFERENCES

Ghosh et al.: "Desulfurization of Coal During Carbonization," Ind. Eng. Chem., 42, 1550-8, August 1950.